

No. 709,482.

Patented Sept. 23, 1902.

A. GUTENSOHN.

PROCESS OF ELIMINATING THE SULFUR FROM SULFID ORES.

(Application filed Feb. 21, 1901.)

(No Model.)



Witnesses.

A. M. Parkins.

E. A. Breeoch.

Inventor.

Adolph Gutensohn,  
By his Attorneys,  
Baldwin, Dandson & Wright

# UNITED STATES PATENT OFFICE.

ADOLPH GUTENSOHN, OF LONDON, ENGLAND, ASSIGNOR TO SULPHUR ELIMINATION SYNDICATE, LIMITED, OF LONDON, ENGLAND.

## PROCESS OF ELIMINATING THE SULFUR FROM SULFID ORES.

SPECIFICATION forming part of Letters Patent No. 709,482, dated September 23, 1902.

Application filed February 21, 1901. Serial No. 43,368. (No specimens.)

*To all whom it may concern:*

Be it known that I, ADOLPH GUTENSOHN, working chemist, a subject of the German Emperor, residing at Crown Works, Park 5 street, Limehouse, London, England, have invented a new or Improved Process of Eliminating the Sulfur from Sulfid Ores, of which the following is a specification.

This invention has for its object the elimination of sulfur from sulfid ores of all kinds—such as pyrites, sulfids of copper, zinc, lead, &c.—and also from ores in which sulfids may be associated with arsenic, tellurium, or other volatile elements, or from artificial products, 15 such as concentrates or mattes. Where arsenic, tellurium, &c., are present, the substances will be eliminated with the sulfur. All methods hitherto used demand a prolonged roasting period and a consumption of 20 a considerable proportion of fuel. Moreover, it is always a matter of extreme difficulty by such methods to eliminate the last portions of the sulfur and to obtain a dead or sweet roast. This difficulty is greater still when 25 arsenic, antimony, or tellurium are present, also blonde and galena. By this process these difficulties are either entirely avoided or greatly minimized. The roasting period is reduced to a small fraction of the time hitherto required, and the sulfur is either completely eliminated, if the process is perfect, or if not, left only in small quantities in the 30 form of soluble or insoluble sulfates of the metals present, which will not interfere with 35 subsequent extraction operations for gold or silver.

The accompanying drawing shows a transverse section of a furnace which may be employed.

According to this invention I mix suitably-crushed iron pyrites, or iron pyrites admixed with other sulfid ores, or sulfid ores without such admixture, with a certain proportion of similarly-powdered carbon or suitable carbonaceous material and add to the mixture or to the carbon, &c., beforehand a further suitable proportion of sodium sulfid, or a mixture of carbon and sodium sulfate, or sodium carbonate, or sodium hydroxid, or such other suitable 45 salt of sodium, as by interaction with carbon and a metallic sulfid, shall be capable of pro-

ducing during the first stage of the operation sulfid of sodium. The mixture is then exposed to a low heat—say approaching incipient redness—for a short time. This time will naturally vary according to the richness of the ore in sulfur and to the fineness to which it has been ground, and may be from a few minutes to, say, half an hour, according to the circumstances of the case. Probably what takes place when 55 the mixture of iron pyrites, sodium sulfid, and carbon are first heated is that a certain amount of carbon disulfid is formed and also sodium polysulfid and the iron reduced to the state of monosulfid of iron. This may be expressed 60 by the following equation:



(Note,  $x$  denoting an excess quantity.) The crystals of  $\text{FeS}_2$  thus become broken down 70 and the  $\text{FeS}$  is left in a minutely-divided condition intimately mingled with finely-divided carbon, which keeps the heated mass in an open porous condition, through which air can freely penetrate. On removing the charge 75 from the source of heat and exposing to air—rabbling, if necessary—or by freely admitting air after this first stage of the operation oxidation proceeds with the greatest rapidity, partly by reason of the mass being already 80 heated to a heat approaching incipient redness, partly by reason of its open porous condition, and partly because the carbon itself becomes oxidized and aids in further heating the mass. The mass becomes heated to a red 85 heat, and the carbon and much of the sulfur are burned off, leaving the iron in the form of red oxid ( $\text{Fe}_2\text{O}_3$ ) and the sodium in the form of sulfate, which can readily be removed and allow of gold, silver, &c., being extracted by 90 any suitable means, such as by chlorination, amalgamation, or by cyanidation. This may be expressed by the following equation:



To heat the mixed ore, carbon, and sulfid of sodium before exposing it to air, the mixed mass may be placed in a layer a few inches deep upon a plate heated by a fire below, and 100 a suitable cover should be placed over the plate to more or less exclude air.

In the drawing, A indicates the plate, B the fireplace below it, and C the cover.

When the mass has become sufficiently heated, the cover may be removed and the mass raked off and exposed to air and rabbled to allow of its oxidation, or it may be allowed to oxidize on the plate, or the preliminary heating might be effected in other forms of furnace in a neutral or reducing flame and subsequently oxidized, or the heating and oxidation may be carried on continuously.

I find that pyrites or mispickel charges which hitherto would have required a calcination period of many hours, even in some cases up to twenty-four hours, can when heated in the manner above described be freed from sulfur and brought to the state of a dead or sweet roast after a period of from, say, one hour to two hours in the furnace, the completion of the oxidation being effected by exposure to the open air.

In view of the wide variations in composition of the ores before mentioned it is not easy to give definite proportions of the materials to be used in every case; but I have found a useful admixture to be the following: Powdered carbon equal to about one-fifth of the total sulfur present with the addition of a suitable sodium salt—say of dry sulfid of sodium ( $Na_2S$ )—which shall be equivalent to about one-fifth of the weight of carbon, or, if a mother-liquor of sodium sulfid crystals be employed, a weight of this equal to half the carbon used. After the reaction is complete the sodium will be found to be present as sodium sulfate, while the carbon has nearly or entirely disappeared. This reaction has the further advantage that it can be used with great efficiency in producing what is known as a “chloridizing roast.” This operation is frequently employed in the treatment of ores which contain sulfid, antimonid, &c., of silver associated with other metallic sulfids. If such an ore be roasted in the ordinary way, with the addition of the requisite quantity of sodium chlorid, the silver is found in the form of chlorid at the end of the roasting operation. The degree of heat and the length of time, however, required under such circumstances give rise to considerable losses of the precious metals as volatilized chlorids, whereas the low temperature and the short period required by my method avoids these serious chloridizing losses. The sodium chlorid required may be added before the commencement of the roast or at any stage prior to the final breaking up of the sulfates.

I do not necessarily bind myself to the proportions given, as it will be evident that a certain minimum proportion of carbon is required even in ores very poor in sulfur, but state the above as an example of the admixture which I have found to be efficacious in the treatment of rich pyritic and arsenical gold ores and concentrates. The gold and silver can be extracted from the residues by

any suitable means, such as by chlorination, amalgamation, cyanidation, &c.

What I claim is—

1. The hereinbefore-described process for the elimination of sulfur from sulfid ores, consisting in crushing the ore, mixing it with carbon and a sodium salt which will yield sulfid of sodium when the mixture is heated, the amount of carbon added being largely in excess of the amount required to form the sulfid of sodium heating the mixture to a temperature approaching incipient redness, and then exposing it freely to air to effect its oxidation and burn off all sulfur that is set free. 70 75 80

2. The hereinbefore-described process for the elimination of sulfur from sulfid ores, consisting in crushing the ore, mixing it with carbon and sodium sulfid, heating the mixture to a temperature approaching incipient redness, and then exposing it freely to air to effect its oxidation and burn off all sulfur that is set free. 85

3. The hereinbefore-described process for the elimination of sulfur from sulfid ores, consisting in crushing the ore, mixing it with crushed iron pyrites, carbon and a sodium salt which will yield sulfid of sodium when the mixture is heated, the amount of carbon added being largely in excess of the amount required to form the sulfid of sodium heating the mixture to a temperature approaching incipient redness, and then exposing it freely to air to effect its oxidation and burn off all sulfur that is set free. 90 95 100

4. The hereinbefore-described process for the elimination of sulfur from sulfid ores, consisting in crushing the ore, mixing it with crushed iron pyrites, carbon and sodium sulfid, heating the mixture to a temperature approaching incipient redness, and then exposing it freely to air to effect its oxidation and burn off all sulfur that is set free. 105

5. The hereinbefore-described process for the elimination of sulfur from sulfid ores, consisting in crushing the ore, mixing it with carbon, sodium chlorid and a sodium salt which will yield sulfid of sodium when the mixture is heated, the amount of carbon added being largely in excess of the amount required to form the sulfid of sodium, heating the mixture to a temperature approaching incipient redness, and then exposing it freely to air to effect its oxidation and burn off all sulfur that is set free. 110 115 120

6. The hereinbefore-described process for the elimination of sulfur from sulfid ores, consisting in crushing the ore, mixing it with carbon, sodium chlorid and sodium sulfid, heating the mixture to a temperature approaching incipient redness, and then exposing it freely to air to effect its oxidation and burn off all sulfur that is set free. 125

7. The hereinbefore-described process for the elimination of sulfur from sulfid ores, consisting in crushing the ore, mixing it with crushed iron pyrites, carbon, sodium chlorid

and a sodium salt which will yield sulfid of sodium when the mixture is heated, the amount of carbon added being largely in excess of the amount required to form the sulfid of sodium, heating the mixture to a temperature approaching incipient redness, and then exposing it freely to air to effect its oxidation and burn off all sulfur that is set free.

8. The hereinbefore-described process for the elimination of sulfur from sulfid ores, consisting in crushing the ore, mixing it with crushed iron pyrites, carbon, sodium, chlorid, and sodium sulfid, heating the mixture to a temperature approaching incipient redness, and then exposing it freely to air to effect its oxidation and burn off all sulfur that is set free.

9. The hereinbefore-described process for the elimination of sulfur from sulfid ores, consisting in crushing the ore, mixing it with carbon and a sodium salt which will yield sulfid of sodium when the mixture is heated, the amount of carbon added being largely in excess of the amount required to form the sulfid of sodium, heating the mixture to a temperature approaching incipient redness, adding sodium chlorid during the heating, and then exposing it freely to air to effect its oxidation and burn off all sulfur that is set free.

10. The hereinbefore-described process for the elimination of sulfur from sulfid ores, consisting in crushing the ore, mixing it with car-

bon and sodium sulfid, heating the mixture to a temperature approaching incipient redness, adding sodium chlorid during the heating, and then exposing it freely to air to effect its oxidation and burn off all sulfur that is set free.

11. The hereinbefore-described process for the elimination of sulfur from sulfid ores, consisting in crushing the ore, mixing it with crushed iron pyrites, carbon and a sodium salt which will yield sulfid of sodium when the mixture is heated, the amount of carbon added being largely in excess of the amount required to form the sulfid of sodium, heating the mixture to a temperature approaching incipient redness, adding sodium chlorid during the heating, and then exposing it freely to air to effect its oxidation and burn off all sulfur that is set free.

12. The hereinbefore-described process for the elimination of sulfur from sulfid ores, consisting in crushing the ore, mixing it with crushed iron pyrites, carbon and sodium sulfid, heating the mixture to a temperature approaching incipient redness, adding sodium chlorid during the heating, and then exposing it freely to air to effect its oxidation and burn off all sulfur that is set free.

ADOLPH GUTENSOHN.

Witnesses:

ROBERT B. RAUSFORD,  
JOHN H. WHITEHEAD.